# EUROPEAN PATENT APPLICATION

(11) **EP 4 776 266 A1**
(43) Date of publication of application: **15.07.2026**
(21) Application number: 24862605.3
(22) Date of filing: 22.08.2024
(51) Int. Cl.: G09F 3/02, G09F 3/00, G09F 3/10

(54) **LABEL**

(30) Priority: 08.09.2023 JP 2023146238
(71) Applicant: Mitsubishi Paper Mills Limited, Tokyo 130-0026 (JP)
(72) Inventor: IKEZAWA, Yoshimi, Tokyo 130-0026 (JP); URASAKI, Jun, Tokyo 130-0026 (JP)
(74) Representative: Vossius & Partner Patentanwälte Rechtsanwälte mbB
(86) International application number: PCT/JP2024/029890
(87) International publication number: WO 2025/052952

(57) **Abstract**

[Problem] Provided are a label that can be affixed to an adherend without defects, and a method for producing the label.

[Solution] The problem can be solved by a label having a paper base material, a recording layer on a front surface of the paper base material, a remoistening active adhesive layer on a back surface of the paper base material, in which a curl value obtained by cutting the label to a size of 80 mm in CD × 80 mm in MD on a basis of the paper base material, leaving the label to stand in an environment of 23°C and a relative humidity of 50% for 24 hours, and measuring the curl value in the same environment after the standing, based on a state in which the remoistening active adhesive layer faces upward, is 0 mm or more and 30 mm or less; and a curl value obtained by subsequently wetting the remoistening active adhesive layer to an extent that the remoistening active adhesive layer exhibits adhesiveness in the same environment, and measuring the curl value after an elapse of 10 seconds from the wetting, based on a state in which the remoistening active adhesive layer faces upward, is -30 mm or more and 0 mm or less.

## Description

### Technical Field

The present invention relates to a label having a remoistening active adhesive layer containing a remoistening active adhesive as an adhesive function.

### Background Art

A label (sticking paper) having a remoistening active adhesive layer on the back surface can be affixed to an adherend after being moistened by, for example, applying water to the remoistening active adhesive layer to exhibit an adhesive function. Since the remoistening active adhesive layer exhibits the adhesive function by being moistened, a label having an adhesive layer has an advantage that a release paper for the adhesive layer, which is usually required for the label, is not required.

In a label in the related art, which has a remoistening active adhesive layer on the back surface and a recording surface on the front surface, a remoistening adhesive is applied to one surface of printing paper, and then a character or a figure is printed on the front surface. The remoistening adhesive side of the label is likely to shrink due to a heat roll during such printing, and furthermore, the printing paper is likely to be extended by humidity in the atmosphere after the printing, and the label is thus likely to be curled. Therefore, in a case where water is applied to the remoistening adhesive, there is a problem that the application of water is difficult during mechanical conveyance. In order to solve the problem, for example, Patent Document 1 discloses sticking paper, in which a remoistening adhesive is applied to one surface of printing paper, and a surface treatment agent for performing various types of printing such as characters or figures is applied to the other surface to form sticking paper, which prevents curling due to extension of the printing paper with respect to the outdoor air humidity.

### Prior Art Document

### Patent Document

Patent Document 1: JP-A-2013-231256

### Summary of Invention

### Problem to be Solved by the Invention

In addition to the problem that curling occurs before the remoistening active adhesive layer is moistened as described above, in a label having a paper base material, a recording layer on a front surface of the paper base material, and a remoistening active adhesive layer on a back surface of the paper base material, there exist other curling occurrence-inducing factors that adversely affect the affixation.

That is, in a case where the remoistening active adhesive layer is moistened by, for example, applying water to the remoistening active adhesive layer in order to exhibit the adhesive function of the remoistening active adhesive layer and then affix the label to an adherend, a difference in expansion and contraction occurs between the front and back surfaces of the label due to the influence of the applied moisture, and as a result, curling occurs in the label. The label in which curling has occurred is difficult to handle, which causes defects in the affixation of the label to the adherend. For example, in a case where curling in which the remoistening active adhesive layer forms the inner side has occurred, wrinkles, edge folding, or the like are likely to occur during the affixing of the label. On the other hand, in a case where curling in which the remoistening active adhesive layer forms the outer side occurs, rolling, edge folding, or the like is likely to occur during the affixation of the label.

An object of the present invention is to provide a label having a paper base material, a recording layer on a front surface of the paper base material, and a remoistening active adhesive layer on a back surface of the paper base material, in which the occurrence of curling caused by the wetting of the remoistening active adhesive layer is suppressed and the label can be affixed to an adherend without defects, and a method for producing such a label.

### Means for Solving the Problem

An object of the present invention can be accomplished by the following.
[1] A label having a paper base material; a recording layer on a front surface of the paper base material; and a remoistening active adhesive layer on a back surface of the paper base material, in which a curl value obtained by cutting the label to a size of 80 mm in CD × 80 mm in MD on a basis of the paper base material, leaving the label to stand in an environment of 23°C and a relative humidity of 50% for 24 hours, and measuring the curl value before moistening the remoistening active adhesive layer, based on a state in which the remoistening active adhesive layer faces upward, in the same environment after the standing is 0 mm or more and 30 mm or less, and a curl value obtained by subsequently wetting the remoistening active adhesive layer to an extent that the remoistening active adhesive layer exhibits adhesiveness in the same environment, and measuring the curl value after an elapse of 10 seconds from the wetting, based on a state in which the remoistening active adhesive layer faces upward, is -30 mm or more and 0 mm or less.
[2] The label according to [1], in which, in a tensile strength determined in accordance with ISO1924-2:1994, a ratio (MD/CD) of a specific tensile strength on an MD side to a specific tensile strength on a CD side is 1.05 or more and 1.75 or less.
[3] The label according to [1] or [2], in which the paper base material contains one, or two or more water-soluble polymer selected from the group consisting of starch and polyvinyl alcohol as a surface sizing agent using a size press.
[4] The label according to any one of [1] to [3], in which a curl value obtained by wetting the remoistening active adhesive layer using an aqueous solvent having an amount of water of 0.5 times or more and 5 times or less with respect to a coating amount (g/m², dry solid content) of the remoistening active adhesive layer in the remoistening active adhesive layer, and measuring the curl value after an elapse of 10 seconds from the wetting, based on a state in which the remoistening active adhesive layer faces upward, is -30 mm or more and 0 mm or less.

### Effects of the Invention

According to the present invention, it is possible to provide a label having a paper base material, a recording layer on a front surface of the paper base material, and a remoistening active adhesive layer on a back surface of the paper base material, in which the occurrence of curling caused by the wetting of the remoistening active adhesive layer is suppressed and the label can be affixed to an adherend without defects, and a method for producing such a label.

### Description of Embodiments

The label of the present invention is a label having a paper base material; a recording layer on a front surface of the paper base material; a remoistening active adhesive layer on a back surface of the paper base material, in which a curl value obtained by cutting the label to a size of 80 mm in CD × 80 mm in MD on a basis of the paper base material, leaving the label to stand in an environment of 23°C and a relative humidity of 50% for 24 hours, and measuring the curl value before moistening the remoistening active adhesive layer, based on a state in which the remoistening active adhesive layer faces upward, in the same environment after the standing is 0 mm or more and 30 mm or less, and a curl value obtained by subsequently wetting the remoistening active adhesive layer to an extent that the remoistening active adhesive layer exhibits adhesiveness in the same environment, and measuring the curl value after an elapse of 10 seconds from the wetting, based on a state in which the remoistening active adhesive layer faces upward, is -30 mm or more and 0 mm or less (hereinafter also referred to as "the label of the present invention").

Here, in the present specification, the front surface and the back surface of the paper base material are used merely for convenience of description to distinguish the sides of the paper base material, and do not indicate a front surface and the back surface depending on the physical or chemical difference of the paper base material. In addition, in the present specification, CD is "a direction orthogonal to a paper-making flow of a paper machine", and MD is "a paper-making flow direction of the paper machine".

Examples of the label of the present invention include a sheet, a tape, a seal, a display article, and receipt or vouchers.

The paper base material in the label of the present invention includes a single paper layer and a laminate of a plurality of paper layers. In some embodiments, the paper base material has a single paper layer. The reason for this is that the paper base material is advantageous from the viewpoint of the production cost of the label of the present invention.

Moreover, the recording layer of the label of the present invention includes a single layer and a laminate of a plurality of layers.

In addition, the remoistening active adhesive layer of the label of the present invention includes a single layer and a laminate of a plurality of layers. In some embodiments, the remoistening active adhesive layer is a single layer. The reason for this is that the paper base material is advantageous from the viewpoint of the production cost of the label of the present invention.

In the label of the present invention, a protective layer known in the related art in the recording material field can be provided on the recording layer within a range in which the effect of the present invention is not impaired. In addition, in the label of the present invention, an interlayer known in the related art in the recording material field may be provided between the paper base material and the recording layer and/or between the paper base material and the remoistening active adhesive layer for the purpose of, for example, improving the adhesiveness of the layer, assisting recording on the recording layer, and assisting the activity of the remoistening active adhesive layer.

As the paper base material, any of machine-made paper obtained by subjecting a paper stock obtained by adding various additives known in the related art in the paper-making field, such as a filler, a sizing agent, a binder, a fixing agent, a retention aids, and a paper strengthener as necessary to a slurry consisting of pulp such as wood pulp and/or non-wood pulp under acidic, neutral, or alkaline conditions, to a paper-making process by a sheet-forming method known in the related art; sizing base paper obtained by subjecting the machine-made paper to a size press treatment with a size press composition containing a surface sizing agent known in the related art in the paper-making field; surface-treated base paper obtained by subjecting the machine-made paper to a surface treatment with a surface treatment composition containing a surface treatment agent known in the related art in the paper-making field; and plain paper obtained by subjecting the machine-made paper, the sizing base paper, or the surface-treated base paper to a calender treatment can be used.

In the paper base material, the surface on which the size press treatment or the surface treatment is performed may be either of both surfaces and one surface of the machine-made paper, and in the case of one surface, the surface may be either of the front surface and the back surface.

The surface on which the calender treatment is performed may be either of both surfaces and one surface of the machine-made paper, the sizing base paper, or the surface-treated base paper, and in the case of one surface, the surface may be either of the front surface and the back surface.

The paper base material also includes coated paper known in the related art in the coated paper field, in which a coating layer containing a pigment and a binder, or a resin layer containing a resin is provided on the machine-made paper, the sizing base paper, the surface-treated base paper, or the plain paper. Further, the paper base material also includes existing woodfree paper, thin paper, linter paper, kraft paper such as bleached kraft paper, unbleached kraft paper, machine glazed paper, single-side laminated paper, reinforced interlayer paper, and flame retardant paper.

Examples of the above-described wood pulp include pulp consisting of wood fibers known in the related art in the paper-making field. Examples of a raw material of the wood fibers include coniferous trees and broadleaf trees. Examples of the wood pulp include chemical pulp, mechanical pulp, and semi-chemical pulp known in the related art in the paper-making field. Examples of the chemical pulp include leaf bleached kraft pulp (LBKP) and needle bleached kraft pulp (NBKP). Examples of the mechanical pulp include groundwood pulp (GP), pressure groundwood pulp (PGW), refiner mechanical pulp (RMP), thermomechanical pulp (TMP), chemithermomechanical pulp (CTMP), and chemimechanical pulp (CMP). Examples of the semi-chemical pulp include chemigroundwood pulp (CGP).

Examples of the above-described non-wood pulp include pulp consisting of non-wood fibers known in the related art in the paper-making field. Examples of the raw material of the non-wood fibers include woody bast fibers such as kozo, mitsumata, and gampi; herbaceous bast fibers such as flax, hemp, and kenaf; leaf fibers such as Manila hemp, abaca, and sisal hemp; gramineous plants such as rice straw, wheat straw, sugarcane bagasse, bamboo, and esparto; and seed hairs such as cotton and linter.

Furthermore, examples of the pulp include waste paper pulp such as deinked pulp (DIP), and pulp obtained by disassembling spoilage generated in a paper mill.

In some embodiments, the paper base material is the machine-made paper, the sizing base paper, the surface-treated base paper, the plain paper, or kraft paper. The reason for this is that the production cost or the strength of the label of the present invention is excellent.

In at least one embodiment, the paper base material is the machine-made paper, the sizing base paper, the surface-treated base paper, or the plain paper. The reason for this is that the production cost of the label of the present invention is excellent.

In at least one embodiment, the paper base material is kraft paper. The reason for this is that the strength of the label of the present invention is excellent.

In at least one embodiment, the paper base material is sizing base paper containing one, or two or more water-soluble polymer selected from the group consisting of starch and polyvinyl alcohol as a surface sizing agent. The reason for this is that a degree of curling of the paper base material used in the label of the present invention can be further suppressed, and the stiffness of the paper base material is increased, whereby wrinkles, edge folding, or the like is less likely to occur during affixation.

The starch are polysaccharides in which glucose is polymerized through a glycosidic bond, and polysaccharides in which a hydroxyl group of glucose in the polysaccharides in which glucose is polymerized through a glycosidic bond is modified by various substituents. Examples of the starch include starch, oxidized starch, enzyme-modified starch, etherified starch, cationic starch, amphoteric starch, dialdehyde starch, esterified starch such as phosphoric acid esterified starch and urea phosphoric acid esterified starch, hydroxyethylated starch, and hydroxybutylated starch.

In the present specification, polyvinyl alcohol is a generic term including general polyvinyl alcohol and various modified polyvinyl alcohol. Examples of the polyvinyl alcohol include polyvinyl alcohol having various degrees of saponification and various average degrees of polymerization, modified polyvinyl alcohol having various functional groups such as a silyl group, a carboxy group, an amino group, and an acetoacetyl group, and modified polyvinyl alcohol in which other monomers such as ethylene are randomly, graftwise, or blockwise introduced.

The label of the present invention may have a laminate film layer between the paper base material and the remoistening active adhesive layer. In this case, the strength of the label of the present invention related to tearing is likely to be improved, and in a case where the label of the present invention is affixed to an adherend and then the information recorded on the recording layer of the label is removed, the laminate film layer functions as a release layer. Thus, the paper base material and the laminate film layer are likely to be released from each other.

Examples of a material constituting the laminate film layer include known resins in the related art, such as biodegradable resins such as polylactic acid and polybutylene succinate; and synthetic resins such as polyethylene and polypropylene. The laminate film layer can be provided between the paper base material and the remoistening active adhesive layer using a known laminator in the related art, such as a dry laminator, a wet laminator, and an extrusion laminator.

The recording layer in the label of the present invention can be a layer capable of recording an image or a layer in which an image has been recorded, and is not particularly limited.

In some embodiments, the recording can be directly performed on a surface of the paper base material constituting the label of the present invention by a printing method and an image recording method, which will be described later, and the recording layer can be formed. In this case, this is advantageous from the viewpoint of the production cost of the label of the present invention. In a case where an image is directly recorded on a surface of the paper base material, the surface of the paper base material concurrently serves as the recording layer, thus constituting the label of the present invention.

Examples of the recording layer as a layer capable of recording an image include layers capable of recording an image by known printing methods and image recording methods in the related art, such as a coating layer for gravure printing, a coating layer for offset printing, a coating layer for letterpress printing, a coating layer for flexographic printing, a thermosensitive recording layer, an ink receiving layer for ink jet printing, a coating layer for thermal transfer image receiving, an image receiving layer for transfer printing, and a coating layer for electrophotographic printing.

In addition, the recording of the image on the recording layer as a layer capable of recording an image may be performed before and/or after the affixation of the label of the present invention to the adherend.

In some embodiments, the recording layer in the label of the present invention is a thermosensitive recording layer. The reason for this is that the thermosensitive recording printer is widely introduced in the market as a printer for a label.

In some embodiments, in the label of the present invention, the recording layer is a thermosensitive recording layer, and a protective layer is provided to impart scratch resistance and/or chemical resistance to the thermosensitive recording layer.

In addition, in some embodiments, in the label of the present invention, the recording layer is a thermosensitive recording layer, and an interlayer for assisting the recording of the thermosensitive recording layer is provided between the paper base material and the recording layer.

In at least one embodiment, the label of the present invention is a label, in which the recording layer is a thermosensitive recording layer, a protective layer is provided to impart scratch resistance and/or chemical resistance to the thermosensitive recording layer, and an interlayer for assisting the recording of the thermosensitive recording layer is provided between the paper base material and the recording layer.

The recording layer as a layer capable of recording an image can be obtained by coating and drying a coating composition for forming the recording layer on a surface of the paper base material using a coating device and a drying device known in the related art.

Examples of the coating device include coating devices known in the related art in the coated paper field, such as an air knife coater, various blade coaters, various bar coaters, various gravure coaters, various lip coaters, various curtain coaters, and various roll coaters. Further, examples of the coating device include various printing methods such as planography, relief printing, intaglio printing, flexography, gravure, and screen printing.

Examples of the drying device include drying devices known in the related art in the coated paper field, such as hot air dryers such as a linear tunnel dryer, an arched dryer, an air loop dryer, and a sign curve air float dryer; infrared heating dryers; and dryers using a microwave, an ultraviolet ray, or the like.

In some embodiments, the recording layer in the label of the present invention is subjected to a calender treatment using a calender device known in the related art in the paper-making field, such as a machine calender, a soft nip calender, a super calender, a multi-stage calender, and a multi-nip calender, for the purpose of uniformizing and smoothing the recording layer.

In some embodiments, a coating amount of the recording layer is 2 g/m² or more and 40 g/m² or less in terms of the dry solid content. The reason for this is that the occurrence of curling in the label of the present invention is easily suppressed. In a case where the label further has an interlayer and/or a protective layer in addition to the recording layer, the coating amount of the layers including the recording layer and a layer other than the recording layer is 2 g/m² or more and 40 g/m² or less in terms of the dry solid content.

Examples of the recording layer as a layer in which an image has been recorded include a layer obtained by laminating, adhering, or bonding a recording material such as recording paper, patterned paper, colored paper, a pattern film, a colored film, decorative paper, a decorative sheet, and an image recording sheet, on which an image has already been formed, on a paper base material.

The laminating, adhering, or bonding of the recording layer as a layer in which an image has been recorded may be performed before and/or after the affixation of the label of the present invention to an adherend.

The remoistening active adhesive layer in the label of the present invention is an adhesive layer in which a remoistening active adhesive contained in the remoistening active adhesive layer exhibits adhesiveness by wetting the remoistening active adhesive layer with water or a water-containing solution (hereinafter also collectively referred to as "aqueous solvent").

The remoistening active adhesive is known in the related art in the pasting field. Examples of the remoistening active adhesive include starch, such as various modified starch such as oxidized starch and esterified starch, and starch; celluloses such as methyl cellulose, carboxymethyl cellulose, hydroxyethyl cellulose, ethyl hydroxyethyl cellulose, and viscose; chloroprene rubber; polyvinyl alcohol, such as various modified polyvinyl alcohol such as a carboxy group-modified polyvinyl alcohol, and polyvinyl alcohol having various degrees of saponification; polyvinyl ethers such as polyvinyl ethyl ether and polyvinyl isobutyl ether; vinyl acetate-based copolymer such as a vinyl acetate-acrylic acid copolymer and a vinyl acetate-methacrylic acid copolymer; and casein, gelatin, dextrin, gum arabic, glue, and polyacrylamide.

The remoistening active adhesive layer can be obtained by coating and drying a coating composition including at least a remoistening active adhesive for forming the layer on a paper base material using a coating device and a drying device known in the related art. The details of the coating device and the drying device are each the same as those of the coating device and the drying device that can be used for forming the recording layer.

In some embodiments, the remoistening active adhesive layer contains various auxiliary agents in addition to the remoistening active adhesive. The reason for this is that the operability during the coating and drying of the coating composition for forming the remoistening active adhesive layer, the weather resistance of the remoistening active adhesive layer, and the like can be improved. Examples of the auxiliary agent include a preservative, an antioxidant, an antifoaming agent, a surfactant, an antifreezing agent, a scale inhibitor, and a coloring agent.

In some embodiments, the coating amount of the remoistening active adhesive layer is 2 g/m² or more and 25 g/m² or less in terms of the dry solid content. The reason for this is that the occurrence of curling in the label of the present invention is likely to be suppressed. In a case where an interlayer or the like is provided on the back surface of the paper base material in addition to the remoistening active adhesive layer, the coating amount of the layers including the remoistening active adhesive layer and the layers other than the remoistening active adhesive layer is 2 g/m² or more and 25 g/m² or less in terms of the dry solid content.

In some embodiments, the label of the present invention includes a paper base material, a recording layer on a surface of the paper base material, and a remoistening active adhesive layer on a back surface of the paper base material, in which the paper base material is machine-made paper, sizing base paper, surface-treated base paper, plain paper, or kraft paper, and the remoistening active adhesive of the remoistening active adhesive layer is one, or two or more selected from the group consisting of starch, polyvinyl alcohol, vinyl acetate-based copolymer, and dextrin. The reason for this is that the paper base material can be easily recovered and separated from the used label of the present invention, and the environmental load due to the disposal can be reduced.

In at least one embodiment, the label of the present invention includes a paper base material, a recording layer on a surface of the paper base material, and a remoistening active adhesive layer on a back surface of the paper base material, in which the paper base material is machine-made paper, sizing base paper, surface-treated base paper, plain paper, or kraft paper; the recording layer is a thermosensitive recording layer; and the remoistening active adhesive of the remoistening active adhesive layer is one, or two or more selected from the group consisting of starch, polyvinyl alcohol, vinyl acetate-based copolymer, and dextrin.

In the label of the present invention, a curl value obtained by cutting the label to a size of 80 mm in CD × 80 mm in MD on a basis of the paper base material, leaving the label to stand in an environment of 23°C and a relative humidity of 50% for 24 hours, and measuring the curl value before moistening the remoistening active adhesive layer, based on a state in which the remoistening active adhesive layer faces upward, in the same environment after the standing is 0 mm or more and 30 mm or less.

In addition, in the label of the present invention, a curl value obtained by cutting the label to a size of 80 mm in CD × 80 mm in MD on a basis of the paper base material, leaving the label to stand in an environment of 23°C and a relative humidity of 50% for 24 hours, wetting the remoistening active adhesive layer to an extent that the remoistening active adhesive layer exhibits adhesiveness in the same environment after the standing and the curl measurement, and measuring the curl value after an elapse of 10 seconds from the wetting, based on a state in which the remoistening active adhesive layer faces upward, is -30 mm or more and 0 mm or less.

In the label of the present invention, the occurrence of curling due to the wetting of the remoistening active adhesive layer can be suppressed by satisfying the curl values, and as a result, the label can be affixed to an adherend without defects. In a case where the curl values cannot be satisfied, the occurrence of curling due to the wetting of the remoistening active adhesive layer cannot be suppressed. As a result, the label causes defects in the affixation onto an adherend. Furthermore, the curl value is a distance between each of four corner vertices of the label, which has been allowed to stand on a horizontal surface under the conditions, and the horizontal surface, and refers to the maximum value among the measured four corner vertices. The expression, after an elapse of 10 seconds from the wetting, is intended to mean that the curl value is measured before the wetting of the remoistening active adhesive layer is diminished by the environmental temperature and the environmental humidity.

Here, the curl value being a positive value means that a curl in which the remoistening active adhesive layer forms the inner side (hereinafter also simply referred to as a "positive curl") occurs. The curl value being a negative value means that a curl in which the remoistening active adhesive layer is directed outward (hereinafter also simply referred to as a "negative curl") occurs. The curl value is measured by allowing the label to stand with the surface forming the inner side of the curl facing upward.

In addition, the expression "the remoistening active adhesive layer is moistened to an extent that the layer exhibits adhesiveness" refers to a state in which an amount of water is applied such that the remoistening active adhesive in the remoistening active adhesive layer can exhibit adhesiveness uniformly over the entire surface of the remoistening active adhesive layer by applying an aqueous solvent to the entire remoistening active adhesive layer.

Such an amount of water required for the wetting to an extent that the remoistening active adhesive layer exhibits adhesiveness uniformly over the entire surface changes depending on the type of the remoistening active adhesive and the coating amount of the remoistening active adhesive layer, but in a case where the amount of water is 0.5 times or more and 5 times or less with respect to the coating amount (g/m², dry solid content) of the remoistening active adhesive layer per unit area, the remoistening active adhesive layer can exhibit adhesiveness regardless of the type of the remoistening active adhesive.

In some embodiments, the amount of water used for "the wetting to an extent that the remoistening active adhesive layer exhibits adhesiveness" is 0.5 times or more and 5 times or less with respect to the coating amount (g/m², dry solid content) of the remoistening active adhesive layer per unit area.

In at least one embodiment, the amount of water used for "the wetting to an extent that the remoistening active adhesive layer exhibits adhesiveness" is 1 time or more and 4 times or less with respect to the coating amount (g/m², dry solid content) of the remoistening active adhesive layer per unit area. The reason for this is that in a case where the amount of water is used, regardless of the type of the remoistening active adhesive, the aqueous solvent can be sufficiently supplied over the thickness direction of the remoistening active adhesive layer, the remoistening active adhesive layer can exhibit adhesiveness sufficiently, and the dripping of the aqueous solvent can be suppressed.

In some embodiments, the label of the present invention is a label having a paper base material, a recording layer on a front surface of the paper base material, and a remoistening active adhesive layer on a back surface of the paper base material, in which a curl value obtained by cutting the label to a size of 80 mm in CD × 80 mm in MD on a basis of the paper base material, leaving the label to stand in an environment of 23°C and a relative humidity of 50% for 24 hours, and measuring the curl value before moistening the remoistening active adhesive layer, based on a state in which the remoistening active adhesive layer faces upward, in the same environment after the standing is 0 mm or more and 30 mm or less, and a curl value obtained by subsequently wetting the remoistening active adhesive layer using an aqueous solvent having an amount of water of 1 time or more and 4 times or less with respect to a coating amount (g/m², dry solid content) of the remoistening active adhesive layer in the remoistening active adhesive layer in the same environment, and measuring the curl value after an elapse of 10 seconds from the wetting, based on a state in which the remoistening active adhesive layer faces upward, is -30 mm or more and 0 mm or less.

In a label in the related art, having a paper base material, a recording layer on a front surface of the paper base material, and a remoistening active adhesive layer on a back surface of the paper base material, in a case where an aqueous solvent is applied to the remoistening active adhesive layer to wet the remoistening active adhesive layer, the remoistening active adhesive layer side of the paper base material stretches due to the influence of the applied aqueous solvent, and a stress due to a difference in expansion and contraction is generated on the front and back surfaces of the paper base material. As a result, the label is likely to generate a negative curl, in which a curl value based on a state in which the remoistening active adhesive layer faces upward is a negative value.

On the other hand, in order to suppress the negative curl, the label of the present invention has a tendency to generate a positive curl, in which a curl value based on a state in which the remoistening active adhesive layer faces upward is a positive value. Since the label of the present invention has a tendency to generate the positive curl, it is possible to offset the stress that causes the negative curl that occurs in a case where the remoistening active adhesive layer is moistened. As a result, in the label of the present invention, in a case where the remoistening active adhesive layer is moistened to an extent that the remoistening active adhesive layer uniformly exhibits adhesiveness over the entire surface, the occurrence of curl is suppressed and the label can be affixed to an adherend without defects.

In some embodiments, in the label of the present invention, in order to make it possible to affix the label to an adherend without defects, a curl value based on a state in which the remoistening active adhesive layer faces upward is in a range of -10 mm or more and 10 mm or less.

Examples of a method for providing the label of the present invention having a tendency to generate the positive curl include a method in which a moisture content and/or a drying state of the front surface and the back surface of the paper base material constituting the label of the present invention is controlled.

In general, the curl of paper is caused by (1) a difference in drying speed or drying state between the front and back surfaces of the paper, (2) a difference in fiber orientation between the front and back surfaces of the paper, (3) a difference in ease of dehumidification or moisture absorption between the front and back surfaces of the paper or a difference in density between the front and back surfaces of the paper, and (4) a difference in shrinkage rate between the front and back surfaces of the paper due to a coating layer. For example, the factor (1) is affected by a dryer part of a paper-making step, the factor (2) is affected by supply of a paper stock in the paper-making step, a J/W ratio (a ratio of a pulp ejection speed to a long-wire speed), a slice slip, and a wire part, the factor (3) is affected by supply of a paper stock in the paper-making step, a J/W ratio, a slice slip, a wire part, a press part, a size press treatment, and a calender treatment, and the factor (4) is affected by the amount of a pigment component, the amount of a resin component, a coating amount, and drying of a layer. Therefore, the curl of paper can be adjusted by controlling these factors. There exists an empirical rule that the curl of paper is "a curl with the surface from which moisture is removed last forming the inner side", or "a curl with the side that dries more slowly forming the inner side". Therefore, from the viewpoint of having a tendency to generate a curl, the effectiveness of the method using the factor (1) using the difference between the front and back surfaces of the drying speed or the drying state in the dryer part is high.

For example, in the dryer part, the calender treatment, or the drying of the layer, by providing a difference in drying temperature between the front and back surfaces of the paper, movement of moisture occurs in the paper thickness direction, and the moisture content on the side of the surface with a higher temperature setting can be relatively lowered. On the surface with a relatively low moisture content, the fibers of the pulp are easily swollen by applying an aqueous solvent to wet the surface. That is, in a case where a state in which the surface with a higher temperature setting faces upward in a case of being moistened is taken as a reference, the paper has a tendency to generate a curl, in which the surface with a higher temperature setting forms the outer side.

In addition, for example, the J/W ratio and/or the slice slip can be adjusted using a long-wire paper machine to perform slow paper-making in the wire part and the dryer part, and the density of the paper on a so-called felt surface side of the dryer part can be made relatively high. On the side with a higher density, the expansion due to the influence of wetting increases since the fibers of the pulp are densely packed. That is, the paper has a tendency to generate a curl, in which the felt surface forms the outer side in a case of being moistened by applying an aqueous solvent.

Examples of methods other than the methods include a method in which an aqueous solvent is applied to and dried on one surface of paper. Paper in which the moisture content of one surface is relatively high by such a method has a tendency to generate a curl in which the one surface forms the inner side in a case of being moistened.

Then, as the paper base material constituting the label of the present invention, whether the paper base material has a tendency to generate a positive curl or a tendency to generate a negative curl is determined by the selection of which surface of the paper obtained above is to be the front surface or the back surface.

In addition, in some embodiments for obtaining the label of the present invention, as a method for providing the label having a tendency to generate a positive curl, there may be a method for producing the label of the present invention, in which an aqueous solvent is applied onto the remoistening active adhesive layer of the label, and the layer is dried to finish the label. As a result, the label of the present invention has a tendency to generate a positive curl, based on a state in which the remoistening active adhesive layer faces upward in a case of being moistened, due to an increase in the relative moisture content of the remoistening active adhesive layer.

In addition, in some embodiments for obtaining the label of the present invention, as a method for providing the label having a tendency to generate a positive curl, there may be a method for producing the label of the present invention, in which firstly, a coating composition for forming a recording layer is coated and dried on the front surface of the paper base material to provide the recording layer, and secondly, a coating composition for forming a remoistening active adhesive layer is coated and dried on the back surface of the paper base material to provide the remoistening active adhesive layer. As a result, the label of the present invention can have a tendency to generate a positive curl, based on a state in which the remoistening active adhesive layer faces upward, by providing the remoistening active adhesive layer later than the recording layer.

In addition, in some embodiments for obtaining the label of the present invention, as a method for providing the label having a tendency to generate a positive curl, there may be the production method of the present invention, in which in a case of paper making of the paper base material, a difference in drying speed or drying state between the front and back surfaces is set in a dryer part of a paper machine, the recording layer is provided on the side where drying is faster, and the remoistening active adhesive layer is provided on the side where drying is slower. As a result, the label of the present invention can have a tendency to generate a positive curl, based on a state in which the remoistening active adhesive layer faces upward, due to a difference in drying state between the front and back surfaces of the paper base material.

As described above, in a case where the moisture content or the drying state is different between the front and back surfaces of the paper, a difference in expansion and contraction occurs in the paper, and a stress due to the difference in expansion and contraction is accumulated in the paper, which causes curling. According to Mr. AKesson, the paper contracts more on a surface having a low evaporation rate, and curls toward the surface. That is, in coated paper having a coating layer on both surfaces, for example, in a case where both-surface coating is performed with intermediate drying, the paper always curls toward the surface that undergoes the final drying (Rolf AKesson, "Moisturizing and Decurling of Coated Papers", JAPAN TAPPI JOURNAL, Vol. 44, No. 12, pp. 1,267 to 1,274, 1990, p. 1,267).

The method for producing a label of the present invention, in which a coating composition for forming a recording layer is coated and dried on the front surface of the paper base material to provide the recording layer, and a coating composition for forming a remoistening active adhesive layer is coated and dried on the back surface of the paper base material to provide the remoistening active adhesive layer, is a method utilizing the AKesson's principle.

In a label having a paper base material, a recording layer on a front surface of the paper base material, and a remoistening active adhesive layer on a back surface of the paper base material, in order to prevent damage to a recording layer during the production, particularly to a recording layer optimized for a printing method and an image recording method, such as a thermosensitive recording layer, an ink receiving layer for ink jet printing, and a coating layer for thermal transfer image receiving, firstly a coating composition for forming a remoistening active adhesive layer is coated and dried on the back surface of the paper base material to provide the remoistening active adhesive layer, and secondly, a coating composition for forming a recording layer is coated and dried on the front surface of the paper base material to provide the recording layer.

Therefore, usually, it is difficult to select a production method in which a coating composition for forming a recording layer is coated and dried on a front surface of the paper base material to provide the recording layer, and a coating composition for forming a remoistening active adhesive layer is coated and dried on a back surface of the paper base material to provide the remoistening active adhesive layer.

In some embodiments, the label of the present invention is a label having a paper base material, a recording layer on a front surface of the paper base material, and a remoistening active adhesive layer on a back surface of the paper base material, in which a curl value obtained by cutting the label to a size of 80 mm in CD × 80 mm in MD on a basis of the paper base material, leaving the label to stand in an environment of 23°C and a relative humidity of 50% for 24 hours, and measuring the curl value before moistening the remoistening active adhesive layer, based on a state in which the remoistening active adhesive layer faces upward, in the same environment after the standing is 0 mm or more and 30 mm or less, a curl value obtained by subsequently wetting the remoistening active adhesive layer to an extent that the remoistening active adhesive layer exhibits adhesiveness in the same environment, and measuring the curl value after an elapse of 10 seconds from the wetting, based on a state in which the remoistening active adhesive layer faces upward, is -30 mm or more and 0 mm or less, and the paper base material contains one, or two or more water-soluble polymer selected from the group consisting of starch and polyvinyl alcohol as a surface sizing agent using a size press.

In at least one embodiment, the label of the present invention has a paper base material, a recording layer on a front surface of the paper base material, and a remoistening active adhesive layer on a back surface of the paper base material, a curl value obtained by cutting the label to a size of 80 mm in CD × 80 mm in MD on a basis of the paper base material, leaving the label to stand in an environment of 23°C and a relative humidity of 50% for 24 hours, and measuring the curl value before moistening the remoistening active adhesive layer, based on a state in which the remoistening active adhesive layer faces upward, in the same environment after the standing is 0 mm or more and 30 mm or less, a curl value obtained by subsequently wetting the remoistening active adhesive layer using an aqueous solvent having an amount of water of 0.5 times or more and 5 times or less with respect to a coating amount (g/m², dry solid content) of the remoistening active adhesive layer in the remoistening active adhesive layer in the same environment, and measuring the curl value after an elapse of 10 seconds from the wetting, based on a state in which the remoistening active adhesive layer faces upward, is -30 mm or more and 0 mm or less, and the paper base material contains one, or two or more water-soluble polymer selected from the group consisting of starch and polyvinyl alcohol as a surface sizing agent using a size press.

In some embodiments, the label of the present invention has a tensile strength determined in accordance with ISO 1924-2: 1994 "Paper and board - Determination of tensile properties - Part 2: Constant rate of elongation method", in which a ratio (MD/CD) of the specific tensile strength on the MD side to the specific tensile strength on the CD side is 1.05 or more and 1.75 or less.

Here, the specific tensile strength is a value obtained by dividing the tensile strength (kN/m) of the label by the basis weight (g/m²) of the label (tensile strength ÷ basis weight), and the numerical value is rounded to the third decimal place.

In a case where MD/CD is 1.05 or more and 1.75 or less, it is possible to suppress "floating" of the label affixed to the adherend, and it is easy to prevent rolling. Here, in the present specification, the "floating" of the label refers to a phenomenon in which an end of the label affixed to the adherend slightly floats before the remoistening active adhesive of the remoistening active adhesive layer is dried and the adhesion is completed in a case of a label having a negative curl.

The tensile strength of the label of the present invention is substantially determined by the tensile strength of the paper base material since the tensile resistance depends on the entanglement of the pulp fibers. The tensile strength of the paper base material is a physical property value known in the related art in the paper-making field, and can be adjusted by a method known in the related art. For example, the tensile strength can be adjusted by controlling the ash content, the density, the paper strength, the pulp type, and the freeness of the base paper, and controlling the J/W ratio, the concentration and amount of the jetted pulp, the dewatering rate of the wire part, and the like in paper-making.

In at least one embodiment, the label of the present invention is a label having a paper base material, a recording layer on a front surface of the paper base material, and a remoistening active adhesive layer on a back surface of the paper base material, in which a curl value obtained by cutting the label to a size of 80 mm in CD × 80 mm in MD on a basis of the paper base material, leaving the label to stand in an environment of 23°C and a relative humidity of 50% for 24 hours, and measuring the curl value before moistening the remoistening active adhesive layer, based on a state in which the remoistening active adhesive layer faces upward, in the same environment after the standing is 0 mm or more and 30 mm or less, and a curl value obtained by subsequently wetting the remoistening active adhesive layer using an aqueous solvent having an amount of water of 0.5 times or more and 5 times or less with respect to a coating amount (g/m², dry solid content) of the remoistening active adhesive layer in the remoistening active adhesive layer in the same environment, and measuring the curl value after an elapse of 10 seconds from the wetting, based on a state in which the remoistening active adhesive layer faces upward, is -30 mm or more and 0 mm or less. In a tensile strength determined in accordance with ISO 1924-2: 1994, the label has a ratio (MD/CD) of the specific tensile strength on the MD side to the specific tensile strength on the CD side of 1.05 or more and 1.75 or less, and the paper base material contains one, or two or more water-soluble polymer selected from the group consisting of starch and polyvinyl alcohol as a surface sizing agent using a size press.

Examples of a material of the adherend to which the label of the present invention is to be affixed include metals, glasses, resins, plastics, leather, paper, composite materials of these materials, and food products. In addition, examples of the form of the adherend include boards, sheets, fabrics, containers, boxes such as corrugated boxes, various packages, packaging articles, packaging packs, packaging bags, and packaging containers.

In some embodiments, the use of the label of the present invention is for applications such as shipping labels, display labels, tag labels, and barcode labels used in the logistics and retail fields, as well as packaging tapes used for sealing corrugated boxes. The reason for this is that in a case of a label having a release paper with respect to an adhesive layer known in the related art, a release work and a disposal work of the release paper are required at a site where the label is used, whereas these works are not required for the label of the present invention. In addition, in a linerless label known in the related art, which has a recording layer on a front surface of the paper base material, a release layer on the recording layer, and a pressure-sensitive adhesive layer on a back surface of the paper base material, printing, additional writing, and/or overlapping affixation cannot be performed later at the use site due to the presence of the release layer on the outermost surface, but the label of the present invention can perform these works.

In water or a water-containing solution (in which the water and the water-containing solution are collectively referred to as an "aqueous solvent") for wetting the remoistening active adhesive layer, the concept of water includes pure water, distilled water, ion-exchanged water, purified water such as reverse osmosis water (RO water) filtered through an RO membrane, raw water such as river water, spring water, groundwater, and well water, as well as purified water obtained by purifying the raw water.

In some embodiments, the water used for wetting the remoistening active adhesive layer is so-called soft water having a low content of mineral components such as calcium ions and magnesium ions. The reason for this is that it is possible to reduce the adhesion of limescale to, for example, a roller, a sponge, a textile, a paintbrush, a brush, and the like, which are used in a method for wetting the remoistening active adhesive layer described below.

In some embodiments, the aqueous solvent contains an antifungal agent and/or a preservative known in the related art. The reason for this is that it is possible to prevent spoilage of the aqueous solvent during storage.

In some embodiments, the aqueous solvent contains a thickener known in the related art. The reason for this is that it is possible to prevent liquid dripping and the like of the aqueous solvent.

In some embodiments, the aqueous solvent contains a drying inhibitor and/or a moisturizer known in the related art, such as glycerin, polyethylene glycol, urea, and a deliquescent inorganic salt. The reason for this is that it is possible to suppress the evaporation of water of the applied aqueous solvent.

In some embodiments, the aqueous solvent contains a coloring agent such as a coloring dye and a coloring pigment. The reason for this is that the wet state of the remoistening active adhesive layer can be visualized.

In some embodiments, the aqueous solvent is heat-retained or heated. The reason for this is that it is possible to prevent the precipitation of the components contained in the aqueous solvent and/or the freezing of the aqueous solvent.

Examples of the method for applying the aqueous solvent to wet the remoistening active adhesive layer include methods known in the related art, such as roller coating of the aqueous solvent, coating of the aqueous solvent with a sponge, a textile, or the like, coating of the aqueous solvent with a paintbrush, a brush, or the like, spray coating of the aqueous solvent, mist or steam spraying of the aqueous solvent, and dropwise addition of the aqueous solvent. The method for wetting the remoistening active adhesive layer may be any of a batch treatment, a sequential treatment, and a continuous treatment.

### [Examples]

Hereinafter, the present invention will be described with reference to Examples, but is not construed as being limited to these Examples. Furthermore, the unit of parts by mass represents a numerical value of the dry solid content or the substantial component amount. The coating amount represents a numerical value of the dry solid content.

### <Paper Base Material (A)>

A paper stock was obtained by adding 0.9 parts by mass of cationized starch and 0.3 parts by mass of an alkyl ketene dimer-based sizing agent to 100 parts by mass of a pulp slurry consisting of 85 parts by mass of LBKP beaten to a CSF freeness of 370 ml and 15 parts by mass of NBKP beaten to a CSF freeness of 370 ml. The paper stock was machine-made using a long-wire paper machine such that the basis weight was 60 g/m², thereby obtaining a machine-made paper.
Subsequently, both surfaces of the machine-made paper were subjected to a size press treatment using a size press composition including oxidized starch as a surface sizing agent, thereby obtaining a sizing base paper. The coating amount of the size press treatment was adjusted to 1.5 g/m² per surface. The obtained sizing base paper was used as a paper base material of a label.

### <Paper Base Material (B)>

A paper stock was obtained by adding 0.9 parts by mass of cationized starch and 0.3 parts by mass of an alkyl ketene dimer-based sizing agent to 100 parts by mass of a pulp slurry consisting of 85 parts by mass of LBKP beaten to a CSF freeness of 370 ml and 15 parts by mass of NBKP beaten to a CSF freeness of 370 ml. The paper stock was machine-made using a long-wire paper machine such that the basis weight was 60 g/m², thereby obtaining a machine-made paper.
Subsequently, both surfaces of the machine-made paper were subjected to a size press treatment using a size press composition including a fully saponified polyvinyl alcohol having an average degree of polymerization of 1,500 as a surface sizing agent, thereby obtaining a sizing base paper. The coating amount of the size press treatment was adjusted to 1.5 g/m² per surface. The obtained sizing base paper was used as a paper base material of a label.

### <Paper Base Material (C)>

A paper stock was obtained by adding 0.9 parts by mass of cationized starch and 0.3 parts by mass of an alkyl ketene dimer-based sizing agent to 100 parts by mass of a pulp slurry consisting of 85 parts by mass of LBKP beaten to a CSF freeness of 370 ml and 15 parts by mass of NBKP beaten to a CSF freeness of 370 ml. The paper stock was machine-made using a long-wire paper machine such that the basis weight was 60 g/m², thereby obtaining a machine-made paper. The obtained machine-made paper was used as a paper base material of a label.

Here, the preparation of the paper base materials (A) to (C) was performed such that the label finally had a desired specific tensile strength while adjusting the concentration and supply amount of the paper stock, the J/W ratio, and/or the slice slip, and adjusting the dewatering rate of the wire part; and the label finally had a desired curl value while suppressing the difference in density between the front and back surfaces of the paper base material in the wire part and the dryer part, and adjusting the difference in moisture content between the front and back surfaces of the paper base material in the dryer part and the calender treatment.

### <Coating Composition for Interlayer>

A coating composition for an interlayer was prepared by dissolving and/or dispersing the following materials in water.

| | |
|---|---|
| Pigment (calcined kaolin) | 1,000 parts by mass |
| Dispersing agent (ammonium polyacrylate) | 1 part by mass |
| Dispersing agent (sodium hexametaphosphate) | 1 part by mass |
| Binder (styrene-butadiene copolymer) | 120 parts by mass |
| Binder (urea-modified phosphoric acid esterified starch) | 60 parts by mass |

### <Coating Composition for Recording Layer>

A thermosensitive recording layer was used as the recording layer.

A coating composition for a thermosensitive recording layer was prepared by mixing and dispersing a dispersion of a color developer and a sensitizer, a dispersion of a dye precursor, a dispersion of a pigment, and an additive, which were obtained by dissolving and/or dispersing the following materials in water.

### <Dispersion of Color Developer and Sensitizer>

| | |
|---|---|
| Electron-accepting color developer (4-hydroxy-4'-isopropoxydiphenylsulfone) | 200 parts by mass |
| Sensitizer (1,2-bis(3-methylphenoxy)ethane) | 200 parts by mass |
| Dispersing agent (sulfonic acid-modified polyvinyl alcohol) | 40 parts by mass |

### <Dispersion of Dye Precursor>

| | |
|---|---|
| Electron-donating dye precursor (3-di-n-butylamino-6-methyl-7-anilinofluoran) | 100 parts by mass |
| Dispersing agent (sulfonic acid-modified polyvinyl alcohol) | 10 parts by mass |

### <Dispersion of Pigment>

| | |
|---|---|
| Calcium carbonate | 300 parts by mass |
| Dispersing agent (ammonium polyacrylate) | 3 parts by mass |
| Binder (fully saponified polyvinyl alcohol) | 200 parts by mass |

### <Additive>

Zinc stearate 80 parts by mass

### <Coating Composition for Remoistening Active Adhesive Layer>

The following materials were dissolved and/or dispersed in water to prepare a coating composition for a remoistening active adhesive layer.

| | |
|---|---|
| Partially saponified polyvinyl alcohol | 100 parts by mass |
| Antifoaming agent (acetylene glycol) | 0.1 parts by mass |

### <Recording Layer>

The surface of the paper base material was coated with the coating composition for an interlayer with the formulation using a bar coater, and dried using a hot air dryer. Subsequently, the interlayer was coated with the coating composition for a thermosensitive recording layer with the formulation using an air knife coater and dried using a hot air dryer. The concentration of the coating composition for a thermosensitive recording layer and the drying conditions were adjusted so that the label finally had a desired curl value.

### <Remoistening Active Adhesive Layer>

The back surface of the paper base material was coated with the coating composition for a remoistening active adhesive layer with the formulation using a blade coater, and dried using a hot air dryer. The concentration of the coating composition for a remoistening active adhesive layer and the drying conditions were adjusted such that the label finally had a desired curl value.

### <Label>

The label was produced by providing an interlayer and a recording layer on a surface of the paper base material, and providing a remoistening active adhesive layer on the back surface of the paper base material. Furthermore, the front surface and the back surface of the paper base material were appropriately selected in consideration of the direction of the curl.

### <Example 1>

Firstly, the coating composition for a remoistening active adhesive layer was coated and dried on the back surface of the paper base material (A). The coating amount of the remoistening active adhesive layer was 15 g/m². Secondly, the coating composition for an interlayer and the coating composition for a thermosensitive recording layer were sequentially coated and dried on the surface of the paper base material (A). The coating amount of the interlayer was 10 g/m². The coating amount of the thermosensitive recording layer was 4 g/m². Next, moisture was applied and dried by spraying steam onto the surface of the remoistening active adhesive layer. Finally, a calender treatment was performed to smooth the thermosensitive recording layer, thereby obtaining a label. In the calender treatment, a difference between the front and back surfaces was not provided in the temperature setting.

### <Examples 2 to 12 and Comparative Examples 1 to 4>

Firstly, the coating composition for an interlayer and the coating composition for a thermosensitive recording layer were sequentially coated and dried on the surface of the paper base material. The coating amount of the interlayer was 10 g/m². The coating amount of the thermosensitive recording layer was 4 g/m². Secondly, the coating composition for a remoistening active adhesive layer was coated and dried on the back surface of the paper base material. The coating amount of the remoistening active adhesive layer was 15 g/m². Next, a calender treatment was performed to smooth the thermosensitive recording layer, thereby obtaining a label. In the calender treatment, a difference between the front and back surfaces was not provided in the temperature setting. The types of the paper base materials used in each of Examples and Comparative Examples are shown in Table 1.

### <Comparative Example 5>

Firstly, the coating composition for a remoistening active adhesive layer was coated and dried on the back surface of the paper base material (A). The coating amount of the remoistening active adhesive layer was 15 g/m². Secondly, the coating composition for an interlayer and the coating composition for a thermosensitive recording layer were sequentially coated and dried on the surface of the paper base material (A). The coating amount of the interlayer was 10 g/m². The coating amount of the thermosensitive recording layer was 4 g/m². Next, a calender treatment was performed to smooth the thermosensitive recording layer, thereby obtaining a label. In the calender treatment, a difference between the front and back surfaces was not provided in the temperature setting.

### [Evaluation]

The label of each of Examples and Comparative Examples was evaluated as follows. The results are shown in Table 1.

### <Curl Value before moistening of Remoistening Active Adhesive Layer (Curl Value A)>

The obtained label was cut out into 80 mm in CD × 80 mm in MD based on the paper base material to obtain a measurement sample for measuring the curl value.

The measurement sample was left to stand in an environment of 23°C and a relative humidity of 50% for 24 hours in a state of being supported at the intersection of the diagonal lines. After the standing, the measurement sample was allowed to stand on a horizontal platform in the same environment such that the curled inner side of the measurement sample faced upward. For the measurement sample that had been allowed to stand, a distance (mm) between each of the four corners of the measurement sample and the horizontal platform was measured. The maximum value of the distance among the four corner vertices was determined for one measurement sample. For each of Examples and Comparative Examples, the maximum value of each of five measurement samples was measured to calculate an average value, and the decimal point was rounded to obtain a curl value. Furthermore, in a case where the remoistening active adhesive layer forms the inner side of the curl, the curl value was defined as a positive curl, and in a case where the remoistening active adhesive layer forms the outer side of the curl, the curl value was defined as a negative curl.

### <Curl Value after Wetting of Remoistening Active Adhesive Layer (Curl Value B)>

For each measurement sample for which the curl value before moistening of the remoistening active adhesive layer had been measured, in an environment of 23°C and a relative humidity of 50%, the entire surface of the remoistening active adhesive layer was moistened by applying tap water (20 ml/m²) at normal temperature (25°C) using a sponge roller type stamp moistener to the remoistening active adhesive layer to an extent that the remoistening active adhesive layer exhibits adhesiveness, and the measurement sample was allowed to stand on a horizontal platform such that the curled inner side of the measurement sample faced upward. After an elapse of 10 seconds from the application of the tap water, for the measurement sample which had been allowed to stand, a distance (mm) between each of the four corners of the measurement sample and the horizontal platform was measured. The maximum value of the distance among the four corner vertices was determined for one measurement sample. For each of Examples and Comparative Examples, the maximum value of each of five measurement samples was measured to calculate an average value, and the decimal point was rounded to obtain a curl value. Furthermore, in a case where the remoistening active adhesive layer formed the inner side of the curl, the curl value was defined as a positive curl, and in a case where the remoistening active adhesive layer formed the outer side of the curl, the curl value was defined as a negative curl.

### <Ratio (MD/CD) of Specific Tensile Strength>

In accordance with ISO1924-2:1994 "Paper and board - Determination of tensile properties - Part 2: Constant rate of elongation method", the tensile strength on the CD side and the tensile strength on the MD side were each measured, and the specific tensile strength on the CD side and the specific tensile strength on the MD side were determined. Here, the specific tensile strength is a value obtained by dividing the tensile strength (kN/m) of the label by the basis weight (g/m²) of the label (tensile strength ÷ basis weight), and the numerical value is rounded to the third decimal place.

Then, the ratio (MD/CD) of the specific tensile strength on the MD side to the specific tensile strength on the CD side was calculated.

### <Affixation to Adherend - Suitability Evaluation>

The label obtained in each of Examples and Comparative Examples was cut out into 80 mm in CD × 80 mm in MD to obtain an affixation sample. Ten affixation samples were given to each of five test subjects. The test subjects moistened the entire surface of the remoistening active adhesive layer of each affixation sample by applying tap water (20 ml/m²) at normal temperature (25°C) using a sponge roller type stamp moistener to an extent that the remoistening active adhesive layer exhibited adhesiveness. Next, the test subjects performed the affixation work of the affixation sample on each of the 500 mm × 500 mm corrugated cardboard paper fixed on a horizontal platform as an adherend while the remoistening active adhesive layer exhibited adhesiveness. The test subjects performed the affixation work of ten affixation samples of each of Examples and Comparative Examples, and performed sensory evaluation according to the following standard.
3 Points: Ten sheets can be easily affixed without defects.
2 Points: Ten sheets can be affixed with no substantial defects, although requiring somewhat more time.
1 Point: Affixation defects occurred in one or more sheets.

Based on the results of the sensory evaluation of the five test subjects, the defects related to the affixation were evaluated according to the following standard. The results are shown in Table 1.

A: Three or more test subjects evaluated 3 points, and no test subject evaluated 1 point.
B: Three or more test subjects evaluated 2 points, and no test subject evaluated 1 point.
C: One test subject evaluated 1 point.
D: Two or more test subjects evaluated 1 point.

### <Affixation to Adherend - Floating Evaluation>

For all the samples on which the affixation work had been performed in the suitability evaluation, the presence or absence of "floating" at the end of the label was checked before the remoistening active adhesive layer was dried, according to the following standard. The results are shown in Table 1.
A: "Floating" was not observed in all the samples.
B: "Floating" was observed in a number of 1 sample or more and 2 samples or less.
C: "Floating" was observed in a number of 3 samples or more and 4 samples or less.
D: "Floating" was observed in a number of 5 samples or more.

**[Table 1]**

| | Type of paper base material | Curl value A (mm) | Curl value B (mm) | Ratio [MD/CD] of tensile strength | Evaluation of affixation to adherend | |
|---|---|---|---|---|---|---|
| | | | | | Affixation suitability | Floating |
| Example 1 | A | 2 | -25 | 1.38 | B | A |
| Example 2 | A | 2 | -27 | 1.35 | B | A |
| Example 3 | A | 10 | -21 | 1.39 | B | A |
| Example 4 | A | 30 | 0 | 1.39 | A | A |
| Example 5 | A | 17 | -4 | 1.39 | A | A |
| Example 6 | A | 2 | -30 | 1.37 | B | A |
| Example 7 | A | 2 | -14 | 1.05 | A | A |
| Example 8 | A | 2 | -16 | 1.75 | A | A |
| Example 9 | A | 1 | -23 | 1.00 | B | B |
| Example 10 | A | 0 | -27 | 2.09 | B | C |
| Example 11 | B | 2 | -24 | 1.44 | B | A |
| Example 12 | C | 9 | -27 | 1.26 | B | A |
| Comparative Example 1 | A | -3 | 15 | 2.2 | C | A |
| Comparative Example 2 | A | 40 | 4 | 2.2 | C | A |
| Comparative Example 3 | A | 26 | 2 | 2.2 | C | A |
| Comparative Example 4 | A | -6 | -35 | 2.3 | D | D |
| Comparative Example 5 | A | -22 | -43 | 2.0 | D | D |

| | | | | | | |
|---|---|---|---|---|---|---|
| Curl value A: Curl value (mm) before moistening of remoistening active adhesive layer Curl value B: Curl value (mm) after moistening of remoistening active adhesive layer | | | | | | |

From the results in Table 1, it was found that Examples 1 to 12 satisfying the configuration of the present invention were labels that could be affixed to the adherend without defects. On the other hand, it was found that Comparative Examples 1 to 5, which did not satisfy the configuration of the present invention, had defects in the affixation work to the adherend.

Primarily, from a comparison between Examples 1 to 8 and Examples 9 and 10, it was found that in a case where the MD/CD ratio of the specific tensile strength of the label was 1.05 or more and 1.75 or less, floating was less likely to occur before the remoistening active adhesive layer was dried in the affixation of the label to the adherend.

Primarily, from a comparison between Examples 1 to 10, Example 11, and Example 12, it was found that in a case where the paper base material contained one, or two or more water-soluble polymer selected from the group consisting of starch and polyvinyl alcohol as the surface sizing agent, and a variation range of the curl before and after the remoistening active adhesive layer was moistened was small. Although this effect was not shown in the above "Affixation to Adherend - Suitability Evaluation" and "Affixation to Adherend - Floating Evaluation", wrinkling, edge folding, and the like were less likely to occur during the affixation, which was preferable as a label.

## Claims

1. A label comprising:
a paper base material;
a recording layer on a front surface of the paper base material; and
a remoistening active adhesive layer on the back surface of the paper base material,
wherein a curl value obtained by cutting the label to a size of 80 mm in CD × 80 mm in MD on a basis of the paper base material, leaving the label to stand in an environment of 23°C and a relative humidity of 50% for 24 hours, and measuring the curl value before moistening the remoistening active adhesive layer, based on a state in which the remoistening active adhesive layer faces upward, in the same environment after the standing is 0 mm or more and 30 mm or less, and
a curl value obtained by subsequently wetting the remoistening active adhesive layer to an extent that the remoistening active adhesive layer exhibits adhesiveness in the same environment, and measuring the curl value after an elapse of 10 seconds from the wetting, based on a state in which the remoistening active adhesive layer faces upward, is -30 mm or more and 0 mm or less.

2. The label according to Claim 1,
wherein, in a tensile strength determined in accordance with ISO1924-2:1994, a ratio (MD/CD) of a specific tensile strength on an MD side to a specific tensile strength on a CD side is 1.05 or more and 1.75 or less.

3. The label according to Claim 1 or 2,
wherein the paper base material contains one, or two or more water-soluble polymer selected from the group consisting of starch and polyvinyl alcohol as a surface sizing agent using a size press.

4. The label according to Claim 1,
wherein a curl value obtained by wetting the remoistening active adhesive layer using water or a water-containing solution having an amount of water of 0.5 times or more and 5 times or less with respect to a coating amount (g/m², dry solid content) of the remoistening active adhesive layer in the remoistening active adhesive layer, and measuring the curl value after an elapse of 10 seconds from the wetting, based on a state in which the remoistening active adhesive layer faces upward, is -30 mm or more and 0 mm or less.
